

Jan. 31, 1928.

D. C. HARE

1,657,622

METHOD OF TREATING ORES

Filed May 26, 1924

2 Sheets-Sheet 1



Witness

John B. Wade

Inventor  
Donald C. Hare.

by Wilkinson & Giusta

his Attorney

Jan. 31, 1928.

D. C. HARE

1,657,622

METHOD OF TREATING ORES

Filed May 26, 1924

2 Sheets-Sheet 2



Fig. 3.

Fig. 2.



Fig. 4.

Witness:

John B. Hader.

Inventor  
Donald C. Hare.

by Wilkinson & Giusta

his Attorneys

## UNITED STATES PATENT OFFICE.

DONALD C. HARE, OF DENVER, COLORADO, ASSIGNOR TO INTERNATIONAL REDUCTION COMPANY, OF DENVER, COLORADO, A COMMON-LAW TRUST.

## METHOD OF TREATING ORES.

Application filed May 26, 1924. Serial No. 715,871.

This invention relates to improvements in methods of treating ores.

One of the primary objects of the invention has been to devise an improved, simple, 5 economic and effective method for the separation and recovery of desired elements, from their ore bearing gangue or veinstone, in the form of metals or salts of metal, the said improvements involving the features of 10 so initially roasting finely divided charges of the metalliferous deposit, in the presence of appropriate reagents and under a vacuum head or suctional force, as to cause the conversion of its metals from their inherent 15 insoluble to a soluble state, in which latter state they are then separated from the waste rock by suitable steps hereinafter appearing.

The foregoing and other objects and advantages, however, will it is believed be so clearly apparent, as incidental to the following disclosure, that it would serve no useful purpose to more fully enlarge upon the same initially, but as the method itself may perhaps be better understood after a disclosure 25 of suitable apparatus or a practical system for carrying forward the steps thereof, it will doubtless be preferable to first describe such means.

It may be said at the outset, however, that although I have illustrated varying modified arrangements, relatively to the roasting furnace unit or assembly, for uses under varying conditions, still the essential steps of the 35 method remain in all instances practically the same.

With these prefacing remarks, therefore, reference will now be immediately had to the accompanying drawings, illustrating 40 certain practical embodiments of such a system or apparatus, in which drawings

Figure 1 is a longitudinal vertical sectional view through one form of roasting furnace unit and a plurality of associated tanks, receptacles or containers, coupled up therewith and with each other, in series, under suctional force or vacuum head control; and Figures 2, 3 and 4 are fragmentary views, 45 of the furnace end of the system, analogous to Figure 1, but respectively illustrating slightly varying modified forms of the furnace unit or assembly.

Referring first to Figure 1, the numeral 5 designates a hopper, or a chute leading from 50 an ore bin, which discharges into the upper

end of a continuously fed or charged furnace, it being observed that the lower wall of the element 5 closes the upper end of the furnace, and its discharge end may project well within the top of the furnace, to provide a substantial space 6 above the body of finely divided ore in the furnace, although this latter feature may not be so essential to this type of furnace as it would be to the types of Figures 2 and 3, wherein an education conduit leads directly from said upper space.

The upper and lower wall portions of the furnace need not be porous, but its intermediate portion or section 7 is formed of 60 freely porous indurated substance, in such a manner preferably as to provide for innumerable minute tortuous air inlets therethrough, to permit of the free filtering of air from the exterior to the interior of the 65 furnace. This could be accomplished by molding the intermediate section of a concrete or cementitious mixture, with salt admixed therein to be thoroughly distributed throughout the mass, and afterwards leaching out the salt particles to provide for the aforesaid porous characteristics.

This porous section 7 of the furnace may also preferably be provided with a plurality of violet ray lamps 8, disposed serially therearound, for purposes hereinafter appearing, the said lamps being mounted in apertures 70 that are closed by the end or disk guard closures 9, which may be of fused silica.

10 and 11 designate pipes for introducing 75 any suitable fluid, such as steam or a desired gas, into association with the charge at the lower end of the furnace, when it is expedient or desirable to do so, and 12 indicates a 80 steam injecting pipe at the top of the furnace 85 for "dusting" purposes, all of these pipes being under valved control as shown.

The lower open end of the furnace is controlled by any automatically functioning continuously discharging means, simply illustrated conventionally by a rotary disk closure 13 which has a conically formed top face, and its bottom face being provided with an annular rack associated with a mechanically operated pawl 14, intermittently actuated to impart a step-by-step rotation to the bottom closure 13, as will be obvious.

In this type of furnace, as will be understood, combustion is started by delivering an initial charge of burning coals on top of a 110

base charge of the ore, then covering the bed of live coals with another charge of the ore, and then plugging the discharge opening of the hopper until the sulphur in the upper charge of ore becomes thoroughly ignited and free burning. Thereafter, the plug is removed from the discharge opening of the hopper, and a continuous supply of fresh ore is delivered at the upper end of the furnace 5 as the mass is continuously discharged at the lower end thereof, continuing combustion being promoted by the sulphurous contents of the incoming ore and the air drawn into the furnace through its intermediate porous 10 wall section 7, the latter owing to a uniform suctional force being established throughout the roasting body of the ore by virtue of an eduction conduit, now to be referred to, which leads or conveys off all arising vapors, 15 products and gases of combustion into association with liquid containing separation tanks, preferably having baffle elements therein, as will later more fully appear.

This eduction conduit pipe embodies a 20 freely porous arm or section 15 projected downwardly within the furnace, being closed at its bottom, and an exteriorly extending non-porous arm or section 16, open at its outer end, adapted to be projected within 25 one of a series of closed tanks or receptacles. The said porous arm 15 may be formed in the manner as suggested with reference to the porous section 7 of the furnace.

The aforesaid receptacles, indicated at 17—35 18—19—20, may each be provided with a covered hand hole opening 21 at their tops, being also provided with outlets illustrated as draw off cocks 22 at their bottoms, while valve controlled air inlets 23 are provided 40 on all but the last tank 20, or even on the last tank if desired, and the employment of these air inlet pipes 23, or their equivalent, often prove to be material factors, in the air regulation control, as will later appear.

The open outer end of the arm 16, of the eduction conduit, is projected to a position slightly above the bottom of the tank 17, while open-ended pipes 24 and 25 provide communication between the upper interior 50 and the lower interior of the immediately preceding and succeeding tanks, respectively, of the series, with the exception that an analogous open-ended pipe 26 only provides communication between the upper interiors of the last two tanks of the series, indicated at 19—20, the last tank 20 simply being a trap or drip receptacle, whereas the other receptacles function as separation, absorption, condensing or precipitation tanks.

The last tank 20 of the series, although it 60 will be understood that any suitable number of tanks 17—18—19 may be employed, is in communication at its upper interior with a vacuum head establishing source, or suctional pressure force, conveniently illus-

tated by the pipe section 27, which may be controlled by a damper 28, coupled with a rotary suction device 29.

Each of the pipes 16—24—25, at their outlet ends, is preferably provided with a lower freely perforated fixed baffle disk 30, or equivalent foraminous element, and with an upper floatative baffle disk 31, the latter being shown as imperforate excepting for a central aperture for slidingly encompassing its complementary pipe support.

The functioning of these baffle disks, and of the various piping described, will later more fully appear, it being understood that the tanks 17—18—19 are maintained partially filled with water, or other suitable treating liquid, as indicated at 32—33—34, while the liquid indicated at 35, in the last tank 20, is merely the result of any moisture trapped against passage through the suction device 29.

In the slightly modified arrangements of Figures 2, 3 and 4, the same elements which are identical with those of Figure 1 are indicated by the same reference numerals and require no additional description, the principles involved in all of the arrangements being substantially the same, although a few minor alterations occur in the actual furnace structures and their direct equipment.

For instance, the only differences between Figures 1 and 3 are that in Figure 3 the furnace wall 36 is not shown as being freely porous and the porous arm 15 of the eduction conduit is omitted, the exteriorly located eduction pipe arm 16 being in direct communication with the space 6 above the charge of ore in the furnace. In this arrangement air is drawn in through the bottom opening of the furnace, but other air admission means could be provided, and in fact the furnace wall could be made freely porous as in Figure 1.

In Figure 2 provision is made for externally applied heat, so that the furnace wall 37 is encompassed by an outer substantially spaced wall 38, forming the combustion space or chamber 39, with the upper portion of the outer wall leading to a stack and with its lower end provided with air inlet openings 40, which may have control means not shown, and the burner openings 41, with which there are associated any suitable type of fuel injector burners, illustrated conventionally as oil burners 42. In this view a chute 43 is shown leading into the top of the furnace, in substitution for a hopper end proper, and like in Figure 3 the inner end of the eduction pipe 16 directly communicates with the space 6 above the charge of ore in the furnace.

All of the furnaces of Figures 1 to 3 are of the continuous feed type, but at Figure 4 the modification embodies an individually charged furnace, supplying a suitable supporting grate for the charge.

In this form, the top of the furnace wall 44 has a charge introducing opening 45, provided with a suitable snug closure, and towards the bottom of the furnace the same is provided with a suitable grate element 46, which may be of a reversible type or otherwise for discharging purposes, a chamber therebelow being supplied with air through a series of inlets 47 that may be damper controlled as at 48.

As in Figures 2 and 3, the inner end of the eduction pipe 16 directly communicates with a space above the charge of ore in the furnace, which space in this instance is designated by the numeral 49, and the inside face of the top wall of the furnace may supply a further series of violet ray lamps 50, in addition to those indicated at 8 as being disposed around the roasting zone, or in substitution thereof.

The discharge ends of the pipes 10 and 11 for introducing suitable fluids, such as steam or gas when desired, into association with the base of the charge of ore, may enter through one or more of the inlets 47, and a steam injector pipe 52, equivalent to the pipe 12 of the other figures, may terminate in a freely perforated ring member 51, disposed within the space 49, providing downwardly disposed jet orifices for equalizing the distribution of moisture above the charge.

In operation, with all of the foregoing arrangements, during the initial stage of the process, the desired metals, elements, compounds thereof, or metalliferous matter generally, undergo the preliminary step of being converted from an insoluble to a soluble state, in the presence of suitable reagents, during the actual roasting operation, as distinguished from being prepared by roasting for subsequent treatment to cause their conversion into a soluble state. These soluble substances are either in the nature of sulphates or chlorides or both, dependent upon the reagents used, and also are either volatilizable or not dependent upon the actual character thereof and the degree of heat applied in the roasting. Furthermore, by my preferred method, a pressure force is maintained through the aforesaid eduction conduit for conveying off, by way of the arm 16, and delivering into association with suitable receiving liquid, as contained for instance in the tanks 17—19, the gases and other volatile products arising from the roasting charge of ore, and this is preferably accomplished by establishing vacuum heads, as it were, above said receiving liquid, by any suitable means, such as the suctional elements 24 to 29 inclusive.

It follows that the volatilized metallic values which go over, in this distilling step, from the furnace through the pipe 16 into the tank 17, become finally separated from their

entrained or entraining permanent gases, the latter being washed out by the liquid contents 32—33—34 and discharging through the suction device 29, and it being particularly emphasized that the said vaporized metallic values are thus recovered or retained in the tanks, owing to their being retarded and absorbed by said liquid, acting as a solvent, or as condensates or precipitates therein, in the form of metals or salts of metal. Condensing and precipitation may be aided in some instances by introducing a cooling medium, such as air, into the tanks by way of the inlets or valved pipe attachments 23; but these valved inlets 23 serve for an even more important function, in that they may be employed to adjust to a nicety the suctional force or vacuum-like heads over the liquid in the tanks, by the slight admission to or the shutting off of air therefrom, thereby more effectively regulating the actual pull of the suction through the charge.

Separation is augmented by the lower foraminous fixed baffles 30 splitting up the vapors and gases, while the upper imperforate floatative baffles 31 divert and retard the flow of the bubbles formed, and thus provide for more effective absorption, condensation, or precipitation of the desired metallic values, as will be apparent, the lines of discharging flow being through the respective pipes 16—24—25, for discharging beneath the lower baffles 30, thence upwardly around and through said foraminous lower baffles, and thence upwardly and along the underneath faces of the upper imperforate baffles 31, escaping peripherally therearound to the spaces thereabove, although some may also escape through the central aperture of each floatative baffle.

As a matter of actual practice, of course, the roasted residue discharged from the furnace may be, and as a matter of fact would be, put through any suitable leaching process for the recovery of its sulphates as well as those chlorides which have not been volatilized. Even in those instances, however, where a larger proportionate recovery is to be obtained by leaching, as may be the case in the treatment of some ores, the auxiliary recovery attained by my method of additionally collecting all vaporized metallic values, which ordinarily would otherwise be lost, becomes a very material factor in point of saving, and hence the commercial success of the process.

The liquid in the tanks 17—18—19 may initially be water, an appropriate acid, a saline solution, or other suitable liquid, but during the process it becomes, owing to the vaporized chlorides deposited therein, a solution of chlorides in water, acid or other suitable liquid, from which separation may be directly effected, or the solution from

these tanks may be deposited in association with the roasted discharge from the furnace, whereupon total recovery of the desired values may be accomplished by leaching in one operation or series of operations.

Regardless of any leaching operations, however, it will be obvious that the recovery of all volatilized metalliferous matter is of the utmost importance, from the highly essential viewpoints of saving and commercial success.

Furthermore, the character of the roasting and the establishing of an evenly coacting suctional force upon the charge being roasted also have much to do with the success of the process, owing to the fact that a thoroughly effective and even roast must be obtained with an equalized distribution of air relatively to or between the particles of crushed ore, as distinguished from separated air channels being formed therethrough and as also distinguished from the air being delivered over upon and, therefore, not being uniformly distributed throughout the charge, whether or not the air delivered over upon the charge, as in the prior art, be compressed air or heated atmospheric air. In my case, the evolution and progress of gases through the charge occurs in evenly balanced or intimately distributed contact with the particles thereof, resulting from the air being introduced into the actual body of the roast and being uniformly drawn therethrough by the action of said suctional force.

Ordinarily, my aim is to employ salt and sulphur as the main reagents, sulphur being contained in most ores in sufficient quantity although it may be supplied thereto if necessary, and thus cause the formation of hydrochloric acid, sulphuric acid, sulphurous acid and free chlorine by the action of steam and heat on the charge. Without steam free chlorine is generated in excess of the other gases which is sometimes desirable.

By this treatment both sulphates and chlorides are formed some of which are soluble in water while others are only soluble in a saturated solution of a suitable salt. For instance lead sulphate is insoluble in any single acid and silver chloride is insoluble in acid whereas both are soluble in a saturated solution of common salt.

Nearly all chlorides are volatile in an atmosphere of chlorine gas or hydrochloric acid gas; but since both sulphates and chlorides are ordinarily formed by the foregoing treatment it is necessary to leach the roasted residue to recover the sulphates therefrom as well as any remaining chlorides, the volatilized chlorides having been conveyed off through the eduction conduit, before described, by virtue of the suctional force maintained therethrough.

If a straight gold ore is to be treated, however, chlorine is wanted almost exclu-

sively; but, as sulphur is nearly always present, the conditions for the evolution of chlorine should be created by the addition of some reagent that forms a third product capable of reacting with the chlorine. Carbon is a suitable agent for this action, carbon tetrachloride being formed, and this action is more favorable than any such action that in its absence, would otherwise produce sulphur chlorides. In this case it would be expected to almost entirely if not wholly volatilize the gold contents, and accordingly a dry charge would preferably be used in any of the furnaces shown.

Where, however, a complex ore is being treated, such as one carrying gold, silver, lead and copper or zinc, it would depend on which of the values predominated, whether or not a greater or lesser degree of volatilization was desired, and also the form under which any or all of the values were wanted. Under such conditions, a fairly high temperature would be maintained, and, if steam is not too plentiful, some of the more volatile chlorides would be vaporized and conducted off; but most of the chlorides would remain in the charge together with the sulphates of the base metals formed, having been converted in the roasting operation itself, however, from their insoluble to a soluble state.

Furthermore, it is believed to be apparent that, in all cases, the action, results and savings attained are superiorly effected where a suctional force is established through the charge, as contemplated by my method, owing amongst other obvious reasons to the reduced pressure in the furnace; and accordingly I claim this feature of converting the metalliferous values, of the roasting mass, from an insoluble to a soluble state, during the actual roasting step, by the employment of suitable reagents and the introduction of air directly into the body of and its uniform distribution throughout said roasting mass, by the application of a suctional force upon the roasting charge, and particularly so where such suctional force is established through the liquid of a liquid containing tank, especially with said suctional force being under regulable air admission and shutting off control at the liquid containing tank zone, for the separation of the metallic values from the volatilized matter drawn off from said charge.

As before suggested, the generation of the treating gases within the charge may be effected by the introduction of salt or calcium chloride, but it is to be understood that there may be added any suitable catalytic agents, such as manganese dioxide, vanadic acid, or cerium nitrate, and it is also to be understood that the treating gases, such as chlorine, or an additional supply thereof, if desired, may be introduced into association with the

charge from an external source, such as by means of one of the pipe lines 10, or 11, the other pipe line being utilized for the supplying of steam as desired. Where the lamps 5 before referred to are employed, the chlorine will be highly activated by the ultra-violet rays emanating therefrom.

The catalytic agents either help the action of these treating gases or break them up with 10 the formation of chlorides and sulphates of the metals, and if the temperature is high enough, with the charge comparatively dry, then the chlorides are more volatile and such as become vaporized will be conveyed off by 15 way of the eduction conduit, as before mentioned, while the discharged roasted residue is subsequently treated by leaching to recover any remaining chlorides and the sulphates contained in association with the discharged 20 material.

Some metals are volatilizable in a stream of hydrochloric acid gas, and for this reason a certain degree of latitude must be exercised in the use of an appropriate mixture that 25 will properly yield the desired treating gases, without the generation of other gases of such volume as to interfere with the desired action. Analogously, other gases may be wanted in excess of chlorine or hydrochloric 30 acid, and salt and sulphur would be used for their generation.

Finally, the actual character of the ore being treated will largely determine the nature and amounts of the reagents to be used, as 35 well as the preferred type of furnace to be employed, to get the maximum results, dependent upon whether the major portion of the metalliferous values are to be volatilized and conveyed off, or are simply to be 40 converted into soluble chlorides and sulphates, during the roasting step, to be recovered by leaching, with only a minor portion of the chlorides becoming actually vaporized and conveyed off, dependent upon 45 the heat applied and other conditions.

Having thus fully disclosed my improved method, and a practical systematic combination of means for carrying forward the steps thereof, it will nevertheless be understood 50 that I do not necessarily confine myself to all of the details exactly as disclosed, excepting as they may come within the terms or tenor of the claims, or equivalent steps, or as fairly interpreted in the light of the specification 55 if necessary.

What I do claim, as new and patentable, is:—

1. A method of treating finely divided ores 60 which embodies the steps of roasting the ore in the presence of appropriate reagent matter while supplying air to the roast over a substantial area at a lower position thereof, and conveying off all volatilized matter, for treatment to recover the desired values thereof, by a suctional eduction force that is so

evenly impressed upon said roast as to cause the treating gases and said air to be uniformly drawn in a permeating distributed manner through the actual interior body of the roast, for more effectively converting metalliferous matter thereof to a soluble state during said roasting step. 70

2. A method of treating finely divided ores which embodies the steps of roasting the ore in the presence of appropriate reagent matter while supplying air to the roast over a substantial area at a lower position thereof, conveying off all volatilized matter, for treatment to recover the desired values thereof, by a suctional eduction force that is so evenly impressed upon said roast as to cause the treating gases and said air to be uniformly drawn in a permeating distributed manner through the actual interior body of the roast, for more effectively converting metalliferous matter thereof to a soluble state during said roasting step, and leaching out the remaining desired values from the residue roasted ore. 80

3. A method of treating finely divided ores which embodies the steps of roasting the ore in the presence of appropriate reagent matter while supplying air to the roast over a substantial area at a lower position thereof, and conveying off all volatilized matter to and through an appropriately closed treating bath, for recovering the desired values of said volatilized matter, by a suctional eduction force that is so evenly impressed upon said roast, through the medium of said bath, as to cause the treating gases and said air to be uniformly drawn in a permeating distributed manner through the actual interior body of the roast, for more effectively converting metalliferous matter thereof to a soluble state during said roasting step. 95

4. A method of treating finely divided ores which embodies the steps of roasting the ore in the presence of appropriate reagent matter while supplying air to the roast over a substantial area at a lower position thereof, conveying all volatilized matter to and through an appropriately closed treating bath, for recovering the desired values of 100

said volatilized matter, by a suctional eduction force that is so impressed upon said roast, through the medium of said bath, as to cause the treating gases and said air to be uniformly drawn in a permeating distributed manner through the actual interior body of the roast, for more effectively converting metalliferous matter thereof to a soluble state during said roasting step, and appropriately treating the residue ore from the roast for recovering the remaining desired values therein. 115

5. A method of treating finely divided ores which embodies the steps of roasting the ore in the presence of appropriate reagent matter while supplying air to the roast over a 130

- 8 substantial area at a lower position thereof, conveying all volatilized matter to and through an appropriately closed liquid treating bath by a suctional eduction force that is so evenly impressed upon said roast as to cause the treating gases and said air to be uniformly drawn in a permeating distributed manner through the actual interior body of the roast, for more effectively converting metalliferous matter thereof to a soluble state during said roasting step, maintaining a vacuum-like head under suctional force over said bath liquid for withdrawing through said liquid the formed permanent gases, as relieved of the desired values retained in said bath, and for maintaining the aforesaid eduction force through said roast, regulating the suctional force of said vacuum-like head by a relative slight admission of air to and the shutting off of air therefrom, and appropriately treating the residue ore from the roast for recovering the remaining desired values therein.
6. A method of treating finely divided ores which embodies the steps of roasting the ore in the presence of appropriate reagent matter while supplying air to the interior body of the roast, conveying all volatilized matter to and through an appropriately closed liquid treating bath by a suctional eduction force established through said roast, maintaining a vacuum-like head under suctional force over said bath liquid for withdrawing through said bath liquid the formed permanent gases, as relieved of the desired values retained in said bath, and for establishing the aforesaid eduction force through said roast, and regulating the suctional force of said vacuum-like head by a relative slight admission of air to and the shutting off of air therefrom.
7. A method of treating finely divided ores which embodies the steps of roasting the ore in the presence of appropriate reagent matter while supplying air to the roast over a substantial area at a lower position thereof, conveying all volatilized matter to and through an appropriately closed liquid treating bath by a suctional eduction force that is so evenly impressed upon said roast as to cause the treating gases and said air to be uniformly drawn in a permeating distributed manner through the actual interior body of the roast, for more effectively converting metalliferous matter thereof to a soluble state during said roasting step, maintaining a vacuum-like head under suctional force over said bath liquid for withdrawing therethrough the formed permanent gases, as relieved of the desired values retained in said bath, and for maintaining the aforesaid eduction force through said roast, regulating the suctional force of said vacuum-like head by a relative slight admission of air to and the shutting off of air therefrom, and leaching out the remaining desired values from the residue roasted ore, the said treating bath with its contents being employed in said leaching step.
8. A method of treating finely divided ores which embodies the steps of roasting the ore in the presence of appropriate reagent matter while supplying air to the roast over a substantial area at a lower position thereof, conveying all volatilized matter to and through an appropriately closed liquid treating bath by a suctional eduction force established through said bath and through said roast by way of said bath.
9. A method of treating finely divided ores which embodies the steps of roasting the ore in the presence of appropriate reagent matter while supplying air to the roast over a substantial area at a lower position thereof, conveying all volatilized matter to and through an appropriately closed liquid treating bath by a suctional eduction force that is so evenly impressed upon said roast as to cause the treating gases and said air to be uniformly drawn in a permeating distributed manner through the actual interior body of the roast, for more effectively converting metalliferous matter thereof to a soluble state during said roasting step, maintaining a vacuum-like head under suctional force over said bath liquid for withdrawing through said liquid the formed permanent gases, as relieved of the desired values retained in said bath, and for maintaining the aforesaid eduction force through said roast, regulating the suctional force of said vacuum-like head by a relative slight admission of air to and the shutting off of air therefrom, and leaching out the remaining desired values from the residue roasted ore, the said treating bath with its contents being employed in said leaching step.
10. A method of treating finely divided ores which embodies the steps of roasting the ore in the presence of appropriate reagents including chlorine gas, while the said chlorine gas is being activated by ultra-violet ray emanations and while supplying air to the interior of the roast, and conveying all volatilized matter to and through an appropriately closed treating bath, for recovering the desired values of said volatilized matter, by a suctional eduction force established through said bath and through said roast by way of said bath.
11. A method of treating finely divided ores which embodies the steps of roasting

the ore in the presence of appropriate reagents including chlorine gas, while the said chlorine gas is being activated by ultra-violet ray emanations and while supplying air to the roast over a substantial area at a lower position thereof, conveying all volatilized matter to and through an appropriately closed liquid treating bath by a suctional force that is so evenly impressed upon said roast as to cause the treating gases and said air to be uniformly drawn in a permeating distributed manner through the actual interior body of the roast, for more effectively converting metalliferous matter thereof to a soluble state during said roasting step, 25

5 to the roast over a substantial area at a lower position thereof, and conveying all volatilized matter to and through an appropriately closed treating bath, for recovering the desired values of said volatilized matter, 10 by a suctional eduction force that is so evenly impressed upon said roast, through the medium of said bath, as to cause the treating gases and said air to be uniformly drawn in a permeating distributed manner through 15 the actual interior body of the roast, for more effectively converting metalliferous matter thereof to a soluble state during said roasting step.

12. A method of treating finely divided ores which embodies the steps of roasting the ore in the presence of appropriate reagents including chlorine gas, while the said chlorine gas is being activated by ultra-violet ray emanations and while supplying air 20 to the roast over a substantial area at a lower position thereof, conveying all volatilized matter to and through an appropriately closed liquid treating bath by a suctional force that is so evenly impressed upon said roast as to cause the treating gases and said air to be uniformly drawn in a permeating distributed manner through the actual interior body of the roast, for more effectively converting metalliferous matter thereof to a soluble state during said roasting step, 25

5 to the roast over a substantial area at a lower position thereof, and conveying all volatilized matter to and through an appropriately closed treating bath, for recovering the desired values of said volatilized matter, 10 by a suctional eduction force that is so evenly impressed upon said roast, through the medium of said bath, as to cause the treating gases and said air to be uniformly drawn in a permeating distributed manner through 15 the actual interior body of the roast, for more effectively converting metalliferous matter thereof to a soluble state during said roasting step.

to the roast over a substantial area at a lower position thereof, conveying all volatilized matter to and through an appropriately closed liquid treating bath by a suctional force that is so evenly impressed upon said roast as to cause the treating gases and said air to be uniformly drawn in a permeating distributed manner through the actual interior body of the roast, for more effectively converting metalliferous matter thereof to a soluble state during said roasting step, 30 maintaining a vacuum-like head under suctional force over said bath liquid for withdrawing through said liquid the formed permanent gases, as relieved of the desired values retained in said bath, and for maintaining the aforesaid eduction force through said roast, and regulating the suctional force of said vacuum-like head by a relative slight admission of air to and the shutting off of air therefrom. 35

40

45 In testimony whereof, I affix my signature.

DONALD C. HARE.